

## UNITED STATES PATENT OFFICE

2,000,582

## COMPOSITION FOR STORAGE BATTERY CONTAINERS

Edward R. Dillehay, Glen Ellyn, and Oliver O. Rieser, Oak Park, Ill., assignors to The Richardson Company, Lockland, Ohio, a corporation of Ohio.

No Drawing. Application September 13, 1930,  
Serial No. 481,801

## 10 Claims. (Cl. 106—31)

Our invention relates to the art of molding storage battery containers or boxes from compositions comprising a bituminous binder, a mineral filler, and fibrous matter, usually of 5 vegetable origin, and it has for one of its objects the provision of a new and improved type of binder in such compositions. More specifically, it is an object of our invention to provide a composition for storage battery containers, 10 which contains both an asphaltic substance and a coal tar pitch, as we shall hereinafter set forth.

We accomplish the objects of our invention by that certain process and in that composition 15 of which we shall now describe an exemplary embodiment.

It will be understood that coal tar pitches are in general relatively hard at ordinary temperatures, but have a high susceptibility factor, which 20 means that they shade off very rapidly upon heating, from a solid to a liquid state. They would be advantageous in the manufacture of storage battery containers for several reasons, among which may be pointed out their relative 25 cheapness, the fact that they contribute usefully to the hardness of the composition at ordinary temperatures, and the fact that their relative fluidity at higher temperatures may be employed usefully to increase the plasticity of the composition 30 at molding temperatures.

However, the use of asphaltic substances in storage battery containers is desirable by reason of the fact that they do not have a high susceptibility factor and shade off comparatively 35 slowly from a solid state to a liquid state upon a rise in temperature. Asphaltic substances therefore increase the binder toughness at all temperatures, diminish the brittleness of the composition at low temperatures, and increase 40 its resistance to distortion at relatively high temperatures. Furthermore, the use of asphaltic substances may be employed to produce in the composition, at mixing temperatures, a relatively non-fluid condition, whereby a better distribution of the fibers therein may be obtained. 45

Difficulty has, however, beset attempts to mix asphaltic substances with coal tar pitch, in that in ordinary methods of mixing, precipitation is encountered and the mix is not homogeneous. 50 We have discovered that over a comparatively very wide range of asphaltic substances to be mixed with coal tar pitch, precipitation can be avoided by mixing the substances together at such temperatures that the viscosity of the two materials will be substantially the same. We

have found that when coal tar pitch and asphaltic substances are mixed together at substantially the same viscosity, no trouble is had with precipitation. The effectiveness of our process varies somewhat with different asphaltic materials. We have encountered isolated instances of asphaltic material which will mix under any conditions satisfactorily with coal tar pitch, and we have also encountered isolated instances of asphaltic material which we have been unable 10 to satisfactorily to mix with coal tar pitch and avoid precipitation; but over the general range of asphaltic materials, we have found that mixing at the same viscosity produces a homogeneous result and avoids difficulties with precipitation. 15

Mixing at the same viscosity may, and usually does imply the mixing of the asphaltic substance maintained at one temperature, with the coal tar pitch maintained at another. The temperature of the two substances is, of course, brought 20 to the same level by the operation of the mixing; but the initial, substantially identical viscosity enables the two materials to go together without difficulty, and the resultant mix is homogeneous, 25 free from precipitation, and can be handled just as a single binder may be handled.

In an exemplary practice, we employ as an asphaltic ingredient, a mixture of 50 parts of an asphalt known as stanolite with 50 parts of gilsonite by weight, fluxed together. After the 30 fluxing operation we maintain this asphaltic binder at a temperature of about 450° Fahrenheit. The coal tar pitch we maintain (in order that it may be at the same viscosity as the asphaltic ingredient) at a temperature of 400° 35 Fahrenheit. In making up a suitable binder for storage battery containers, we take 70 parts of the stanolite-gilsonite mixture, having by way of example, the following characteristics:

M. P. 225° F.  
Pen. (150° F.—5 sec.—100 gms.)—20

and holding it, prior to mixing, at a temperature of 450° Fahrenheit, we then mix it with 30 parts of coal tar pitch at a temperature of 45° 400° Fahrenheit. The pitch may have the following characteristics:

Melting point 220—240.

The mixing may be carried on in any suitable 50 vessel, such as a still, or the like, or a mixing machine. If, however, the two materials be put together at approximately identical temperatures, precipitation will occur, and the binder will not be homogeneous.

We manufacture storage battery containers in an exemplary procedure, having a formula comprising 58 parts of combined asphalt and coal tar pitch binder hereinabove described, 30 parts of mineral filler, and 12 parts of fiber. As a mineral filler we prefer to use a diatomaceous earth of acid-resistant character known as Celite. Other mineral fillers are also suitable. They should preferably be acid-resistant in their character; and if they are not porous like diatomaceous earth, they will tend somewhat to increase the specific gravity of the resultant molded composition. We employ as our fibrous ingredient, cotton fibers, such as linters or the like, although other fibers of vegetable or mineral origin may be employed with good results. If the fiber employed is not of acid-resistant character, and if it is of vegetable origin, it should not be employed in amounts greater than 15% by weight of the finished composition. The materials are put together in a mixer, to the extent of homogeneously distributing the fibrous and mineral materials throughout the binder, the binder preferably being in other than a thinly liquid condition. The composition thus formed is usually weighed out into batches and introduced into a mold, where it is molded by hydraulic pressure to form a storage battery container or other article.

Having thus described our invention, what we claim as new and desire to secure by Letters Patent, is:—

1. In a process for the manufacture of bituminous compositions, a binder forming step comprising the initial maintenance of an asphalt component at a temperature to produce a certain viscosity, and the initial maintenance of a coal tar pitch component at a different temperature, to secure the same viscosity therein, and the mixing of the components together while at the same viscosity.

2. In a process for the manufacture of bituminous compositions, a binder forming step which comprises mixing together a coal tar pitch component and an asphalt component, the said components being at initially different temperatures, but having substantially the same viscosity.

3. In a process for the manufacture of bituminous compositions, a binder forming step which comprises mixing together an asphaltic constituent comprising gilsonite and a blown oil, at one temperature, and a coal tar pitch at a different temperature, the temperatures being such that the viscosities of the said components are substantially the same.

4. In a process for making a bituminous composition, the step of mixing together an asphaltic binder component comprising a mixture of stanolite and gilsonite, at about 450° Fahrenheit, and a pitch component at approximately 400° Fahrenheit.

5. A process of making a composition for storage battery cases, which comprises blending together 50 parts of stanolite asphalt and

50 parts of gilsonite to produce an asphaltic binder component, and blending said asphaltic binder component with a coal tar pitch binder component in the ratio of 70 parts of the asphaltic component with 30 parts of the coal tar pitch, the said blending being accomplished while the components are at substantially the same viscosity, and mixing with said binder, to the extent of homogeneous distribution, a mineral filler and a fibrous reinforcement.

6. A process of making a composition for storage battery cases, which comprises blending together 50 parts of stanolite asphalt and 50 parts of gilsonite to produce an asphaltic binder component, and blending said asphaltic binder component with a coal tar pitch binder component in the ratio of 70 parts of the asphaltic component with 30 parts of the coal tar pitch, the said blending being accomplished while the components are at substantially the same viscosity, and mixing with said binder, to the extent of homogeneous distribution, a mineral filler and a fibrous reinforcement, said fibrous material being cotton, and present in amounts not greater than 15% of said composition.

7. A process of making a composition for storage battery cases, which comprises blending together 50 parts of stanolite asphalt and 50 parts of gilsonite to produce an asphaltic binder component, and blending said asphaltic binder component with a coal tar pitch binder component in the ratio of 70 parts of the asphaltic component with 30 parts of the coal tar pitch, the said blending being accomplished while the components are at substantially the same viscosity, and mixing with said binder, to the extent of homogeneous distribution, a mineral filler and a fibrous reinforcement, the said composition comprising 6 parts of binder, 3 parts of mineral filler, and 1 part of cotton fiber.

8. In a process of making plastic bituminous compositions, the steps of controlling the temperature of an asphaltic binder component and controlling the temperature of a coal tar pitch component to bring said components to the same viscosity, and mixing said components together while said compounds have initially the same viscosity.

9. A composition for storage battery containers comprising a mixture of asphalt and coal tar pitch, mineral filler and fibrous reinforcement, the binder component of said composition being characterized as such by more than 25% of both named components, and by homogeneity and an absence of precipitation.

10. A molded product comprising substantially 6 parts by weight of a binder comprising a mixture of coal tar pitch and asphalt, there being present in the mixture as such more than 25% of each component, which mixture is homogeneous in its character and free from precipitation, 3 parts of diatomaceous earth, and 1 part of cotton fiber.

EDWARD R. DILLEHAY.  
OLIVER O. RIESER.